

Patented June 15, 1926.

1,589,062

# UNITED STATES PATENT OFFICE.

JOSEPH ERNST FLETCHER, OF DUDLEY, AND HORACE JOHN YOUNG, OF WHITLEY BAY, NORTHUMBERLAND, ENGLAND.

## IRON CASTING.

No Drawing. Application filed March 18, 1926, Serial No. 95,764, and in Great Britain October 1, 1924.

This invention relates to iron castings to form machine and engine parts, and for other purposes, and has for its object the production of said castings in such manner as will ensure homogeneity, toughness, close grain, and resistance to wear attrition, abrasion or erosion, together with high tensile strength and capacity to withstand shocks or suddenly applied loads at normal or elevated temperatures and pressures.

The invention comprises the manufacture of iron castings in the manner hereinafter described.

The iron we employ in our castings contains preferably less than 3.5 per cent of carbon, but the other elements may be in the proportions commonly found in commercial cast irons though preferably in less proportions than those associated with the production of soft or easily machinable castings.

The internal structure or physical condition of the iron we propose to employ in our castings before treatment is that known as hypoeutectic, the mass of its ferrous grains being more or less embedded in a meshwork consisting mainly of iron and other carbides and phosphides, whilst graphitic carbon is present as flakes or nodules of preferably small dimensions.

In the making of our castings these are cast and cooled, either in moulds of sand, plaster, plumbago, graphite or other like refractory materials including in some cases the use of chills and in others the use of warm or hot moulds, or in moulds such as those made of iron, steel or other metals which are usually preheated. The composition of the cast iron is regulated and additions of other metals or metalloids may be made, in order to favour the production of metal in which the pearlitic condition predominates.

Further, the castings are, if necessary reheated in order to obtain or complete the predominantly pearlitic condition. The reheating may be effected by immersion of the castings in molten metal or molten salts.

The pearlitic or predominantly pearlitic casting so obtained is next reheated either by ordinary means or by immersion in molten metal or molten salts, to a temperature above the critical temperature associated with the formation of pearlite and known as  $Ac_1$ , and then quickly cooled with air, oil,

water, steam or other cooling medium, such as molten metal or molten salts, whereby the structure of the metal is converted to that known as austenitic or partly austenitic—a condition in which the carbon or carbides are considered to be dissolved more or less homogeneously in the iron which, at the temperature or temperature range used for cooling is said to be in the gamma condition.

The casting in the said austenitic condition is then reheated to a temperature not exceeding and preferably below the aforesaid critical change point denoted  $Ac_1$  and quickly cooled. The reheating may be effected in either of the following ways:

(1) The molten metal or salts together with the casting immersed therein are reheated to a temperature not exceeding and preferably below the said critical change point  $Ac_1$ . The casting is then withdrawn from the molten metal or salts and cooled.

(2) The casting alone, after withdrawal from the molten metal or salts is reheated to the extent aforesaid and cooled. Such reheating and recoolings may be accomplished by immersion in other baths of molten metal or salts of suitable temperature, or by other means.

Such treatment produces a further modification of the metal structure in that the ferrous grains take up the conditions known in ferrous metallurgy as sorbitic, troostitic, or martensitic, which give the characteristics of toughness and effective resistance to shocks. Or, the two aforesaid treatments for the production, first of the austenitic or partly austenitic and, second, of the sorbitic or other structure may be combined in another way thus:—The casting in the predominantly pearlitic condition first produced during the primary casting or by means of a further reheating as aforescribed is reheated to above the critical point  $Ac_1$ , but instead of being completely cooled down from such temperature it is quenched briskly in the cooling medium and removed therefrom whilst retaining sufficient heat to bring about the desired structure aforesaid without the necessity for the third operation or treatment as hereinbefore described.

It is known that the said structures are occasionally produced partially in cast iron, unintentionally, but the sorbite, martensite

- and troostite present are heterogeneously mixed with other constituents which destroy the tough condition sought for. By our invention we produce a predominantly sorbitic, troostitic or martensitic or combined structure of uniform character throughout the mass of the ferrous grains of the castings formed as aforesaid from irons of preferably hypoeutectic composition.
- 10 To facilitate the formation of the desired structure there may be used in the mixtures from which the castings are made additions of such other metals or metalloids as will, without preventing the formation of the pearlitic structure by the primary treatment or treatments, promote the formation of the austenitic and sorbitic or troostitic conditions or structures by the second or third treatments or operations.
- 15 Thus, for example, nickel, cobalt, molybdenum, tungsten, vanadium, boron, or chromium may be used for such purpose.
- Having thus described our invention what

we claim as new and desire to secure by Letters Patent is:—

25

1. A process for the production of cast iron castings which comprises forming a casting with a predominately pearlitic structure, transforming said pearlitic structure into austenitic structure and decomposing 30 said stable austenitic structure to a form intermediate pearlite and austenite.

2. A process for the production of cast iron casting which comprises forming a casting with a predominately pearlitic structure, 35 heating said casting to above the  $Ac_1$  point, cooling said casting so as to form stable austenitic structure, reheating said casting to the  $Ac_1$  point as a maximum and cooling said casting so as to decompose said 40 austenitic structure to a form intermediate pearlite and austenite.

In testimony whereof we have signed our names to this specification.

JOSEPH ERNST FLETCHER.  
HORACE JOHN YOUNG.